

June 2, 1942.

**E. M. MARKS**

2,285,294.

## TREATMENT OF HYDROCARBONS

Filed June 11, 1940



*Inventor*  
*Ernest M. Marks*

By *J. Wallace Dunn*  
Attorney

## UNITED STATES PATENT OFFICE

2,285,294

## TREATMENT OF HYDROCARBONS

Ernest M. Marks, Lansdowne, Pa., assignor to  
The Atlantic Refining Company, Philadelphia,  
Pa., a corporation of Pennsylvania

Application June 11, 1940, Serial No. 339,846

7 Claims. (Cl. 196—52)

The present invention relates to the treatment of hydrocarbons, and more particularly to the conversion of hydrocarbons into more valuable products by catalytic reactions involving cracking, reforming, dehydrogenation and polymerization.

It is an object of this invention to convert high boiling hydrocarbon oils into lower boiling hydrocarbons, particularly gasoline. Hydrocarbon oils such as gas oil, heavy distillates, petroleum residuum, tars, and the like may be advantageously converted in accordance with this invention.

It is a further object of this invention to improve the antiknock qualities of gasoline or naphtha distillates and to increase the lead susceptibility thereof by subjecting such distillates to reforming conditions of temperature and pressure in the presence of a catalyst. Such reforming operation involves essentially a dehydrogenation and structural rearrangement of the distillate molecules, with or without cracking and change in boiling range or volatility of the reformed distillate.

In accordance with the present invention, hydrocarbons are subjected to elevated temperatures, under atmospheric or super-atmospheric pressure, in the presence of a catalyst capable of promoting the conversion or reforming reaction, such catalyst comprising aluminum oxide and an alkali metal borate. In the conversion of high boiling oils, such as gas oil, into gasoline, temperatures of the order of from about 850° F. to 1050° F. and pressures up to about 3000 lbs./sq. in. may be employed, while in the reforming of gasoline or naphtha distillates for the improvement of the antiknock quality thereof, temperatures of the order of 975° F. to 1100° F. and pressures of the order of from atmospheric to about 1500 lbs./sq. in. may be advantageously utilized. The reaction time or space velocity may be varied, depending upon the temperature-pressure conditions and the results desired. In general the contact time or space velocity may be somewhat longer in the conversion of high boiling oils into lower boiling hydrocarbons such as gasoline, than in the reforming of gasoline or naphtha distillates for the improvement in antiknock quality thereof. For example, in cracking high boiling oils, the space velocity may be of the order of 1 volume of charge oil per volume of catalyst per hour, whereas in the reforming of distillates, the space velocity may be of the order of 1.5 to 4 volumes of charge oil per volume of catalyst per hour.

The catalyst to be employed in accordance with this invention comprises aluminum oxide or bauxite which has been impregnated with an alkali metal borate. Such catalyst may be prepared by soaking granular aluminum oxide with

an aqueous solution or suspension of an alkali metal borate and thereafter drying the impregnated granular material by heating. Or, alternatively, finely divided aluminum oxide may be impregnated with an alkali metal borate solution or suspension, and the moist material thereafter granulated or formed into suitable pellets or masses. The quantity of borate to be employed may vary from about 0.1% to 10% or more by weight of the aluminum oxide, quantities of the order of from about 1% to about 5% being preferred. Among the borates which may be utilized are the metaborates, tetraborates, penta-borates, hexaborates, octaborates and dodeca-borates of sodium, potassium and lithium.

My invention may be further illustrated with reference to the accompanying drawing, which shows diagrammatically a system suitable for carrying out my process.

Hydrocarbon oil, such as gas oil, is supplied from a source (not shown) through valve-controlled pipe 1 and is passed by means of pipe 2 to heat exchanger 3, wherein the oil is preheated by indirect heat exchange with cracked products from the catalytic chamber hereinafter described. The preheated oil is passed from heat exchanger 3 through pipe 4 to pump 5, from which it is delivered to the tubular heating coil 6 wherein the temperature of the oil is raised to about 950° F., under a pressure of from about 25 to about 50 lbs./sq. in. Higher pressures, of course, may be used. In the coil 6 the oil is vaporized and the heated vapors are passed therefrom by means of pipe 7 into the upper section of catalyst chamber 8 containing a granular catalyst 9 comprising  $\text{Al}_2\text{O}_3$  impregnated, for example, with 1% by weight of sodium borate ( $\text{Na}_2\text{B}_4\text{O}_7$ ). In the chamber 8 cracking of the heated oil in contact with the catalyst takes place, with the production of hydrocarbon gases,  $\text{H}_2$ , cracked gasoline and gas oil, and small amounts of tar. The cracked products, at a temperature of the order of 950° F., are withdrawn from the lower section of chamber 8 and are passed by means of pipe 10 through heat exchanger 3 in indirect heat exchange with relatively cool charge oil introduced through valve-controlled pipe 1 and pipe 2. In the exchanger 3 the hot, cracked products are partially cooled, and thence delivered by valve-controlled pipe 11 to fractionating column 12 provided with contacting plates or trays 13, heating coil 14 and cooling or reflux coil 15. The cracked products are fractionated in column 12 to produce an overhead fraction comprising cracked gasoline and gases, and a bottoms fraction or residue comprising cracked gas oil and small amounts of tar. The cracked gas oil and tar may be withdrawn from the bottom of column 12 by means of valve-controlled pipe 16, and at least a portion thereof

may be recycled, with fresh charge oil, to the tubular heating coil 6. The remainder of the cracked gas oil and tar may be withdrawn from the system through valve-controlled pipe 17 and disposed of as desired.

The gasoline vapors and gases are passed from the top of fractionating column 12 and are introduced by means of pipe 18 into a second fractionating column 19 provided with contacting trays 20, heating coil 21, and cooling coil 22.

following examples, which, however, are not intended as limiting the scope thereof.

The results given in table were obtained by cracking, in a single pass at atmospheric pressure, various gas oils under the conditions and with the catalysts substantially as set forth. The borate-containing catalysts were prepared by impregnating granular  $Al_2O_3$  with aqueous solutions of sodium borate and drying the impregnated granules.

| Gas oil                                      | Catalyst                            | Cracking conditions |                        | Products                      |                    |
|----------------------------------------------|-------------------------------------|---------------------|------------------------|-------------------------------|--------------------|
|                                              |                                     | Tempera-ture, °F.   | Contact time, sec-onds | Volume percent gasoline yield | Weight percent gas |
| Gravity 33.8°; boiling range 353° F.-698° F. | None                                | 1,006               | 7.1                    | 19.4                          | 8.3                |
|                                              | Granular $Al_2O_3$                  | 1,010               | 5.8                    | 32.0                          | 19.0               |
|                                              | Granular $Al_2O_3$ +1% $Na_2B_4O_7$ | 1,006               | 6.0                    | 36.9                          | 19.3               |
|                                              | Granular $Al_2O_3$ +5% $Na_2B_4O_7$ | 1,008               | 6.1                    | 37.9                          | 19.4               |
| Gravity 36.7°; boiling range 300° F.-596° F. | None                                | 1,010               | 6.2                    | 9.4                           | 6.9                |
|                                              | Granular $Al_2O_3$                  | 1,004               | 6.9                    | 22.9                          | 14.6               |
|                                              | Granular $Al_2O_3$ +1% $Na_2B_4O_7$ | 1,006               | 6.5                    | 24.5                          | 15.6               |
|                                              | Granular $Al_2O_3$ +5% $Na_2B_4O_7$ | 1,006               | 6.4                    | 25.9                          | 15.7               |
| Gravity 31.9°; boiling range 220° F.-712° F. | None                                | 1,010               | 6.0                    | 18.0                          | 8.8                |
|                                              | Granular $Al_2O_3$                  | 1,006               | 6.4                    | 28.2                          | 20.7               |
|                                              | Granular $Al_2O_3$ +1% $Na_2B_4O_7$ | 1,006               | 6.5                    | 31.4                          | 21.1               |
|                                              | Granular, fused $Na_2B_4O_7$        | 1,010               | 6.6                    | 18.5                          | 13.1               |

Herein the gases are separated from the gasoline and the latter is stabilized to obtain the desired boiling range and volatility. The stabilized gasoline may be withdrawn from the bottom of the column and passed by means of valve-controlled pipe 23 to storage (not shown). If desired, a liquid side stream comprising  $C_4$  and/or  $C_3$  hydrocarbons may be removed from the column through valve-controlled pipe 24, or  $C_4$  and/or  $C_3$  hydrocarbons may be withdrawn with the uncondensed gases, i. e.,  $C_1$ - $C_2$  hydrocarbons and  $H_2$ , from the top of the column by means of valve-controlled pipe 25. If desired, at least a portion of the uncondensed gas and/or  $C_3$ - $C_4$  hydrocarbons may be recycled to the tubular heating coil 6 by means of valve-controlled pipe 26, compressor 27 and pipe 28.

In the operation of the catalyst chamber 8, the activity of the catalyst may be maintained or increased by the introduction of gases such as steam, oxygen, or carbon dioxide, or mixtures thereof, by means of valve-controlled pipe 29. And at such time as the granular catalyst 9 becomes fouled with carbon or tarry matter, the conversion system may be shut down and the catalyst regenerated by contacting with air or steam at elevated temperatures. Such revivifying agents may be introduced into chamber 8 through valve-controlled pipe 29 and may be withdrawn therefrom, together with the matter contaminating the catalyst, by means of valve-controlled pipe 30.

The reforming of gasoline or naphtha distillates for the improvement of antiknock quality may be carried out in a manner similar to that above described in connection with gas oil cracking. In the reforming operation, it is advantageous to employ somewhat higher temperatures, pressures, and rates of flow than are utilized in the conversion of high boiling oils such as gas oil. Depending upon the nature of the distillate to be reformed, the operating conditions may be varied in order to accomplish reforming with a controlled amount of cracking, or with substantially no cracking, as may be desired.

My process may be further illustrated by the

From the above results, it will be seen that considerably higher yields of cracked gasoline are produced by employing  $Al_2O_3$ - $Na_2B_4O_7$  catalysts of the present invention, than are obtained under similar conditions without any catalyst, or with catalysts such as  $Al_2O_3$  or fused  $Na_2B_4O_7$ , per se.

In order to demonstrate the advantages of employing the  $Al_2O_3$ - $Na_2B_4O_7$  catalysts in the reforming of gasoline for the improvement of the antiknock value and particularly the lead susceptibility thereof, the following examples are presented. A reformer stock, i. e., naphtha distillate was vaporized and passed, at atmospheric pressure, through a chamber containing, respectively, no catalyst,  $Al_2O_3$  catalyst, and

#### $Al_2O_3$ - $Na_2B_4O_7$

catalyst, in three successive runs, the reformed gasoline being condensed and separated from the by-product gas. The operating conditions and the results obtained are shown in the following table.

|                                                               | Catalyst |       |           |                               |
|---------------------------------------------------------------|----------|-------|-----------|-------------------------------|
|                                                               | None     | None  | $Al_2O_3$ | $Al_2O_3$ +5%<br>$Na_2B_4O_7$ |
| Temperature, °F.                                              | 1,050    | 990   | 990       | 1,002                         |
| Contact time, seconds                                         | 6.8      | 7.7   | 7.7       | 6.5                           |
| Gas formed, weight percent                                    | 7.4      | 6.4   | 6.4       | 7.3                           |
| Gasoline, do                                                  | 87.9     | 89.7  | 89.7      | 92.7                          |
| Gasoline, volume percent                                      | 88.4     | 90.9  | 90.9      | 94.3                          |
| Gasoline, A. P. I. gravity degrees                            | 49.3     | 50.5  | 51.4      | 52.3                          |
| Gasoline, percent sulfur                                      | 0.231    | 0.150 | 0.03      | 0.06                          |
| Gasoline, octane number (motor method)                        | 65       | 68    | 68        | 69                            |
| Gasoline, cc. Pb Et <sub>4</sub> to raise to 76 octane number | 6+       | 3.5   | 3.5       | 1.35                          |
| Used catalyst—weight percent carbon deposited                 | None     | 0.70  | 0.70      | 0.27                          |

The reformed gasoline from the  $Al_2O_3$ - $Na_2B_4O_7$  treatment not only had a much higher tetraethyl lead susceptibility than that produced either by straight thermal reforming or reforming in the

presence of  $\text{Al}_2\text{O}_3$ , but the yield was also substantially higher. Furthermore, considerably less carbon was deposited upon the  $\text{Al}_2\text{O}_3\text{-Na}_2\text{B}_4\text{O}_7$  catalyst than upon the  $\text{Al}_2\text{O}_3$  used alone under substantially the same conditions, thereby permitting the former to remain catalytically active for longer periods of time than the latter.

As will be seen from the foregoing, the processes which I have devised utilizing my aluminum oxide-alkali metal borate catalyst are particularly adapted to the manufacture of gasoline, and I therefore prefer to use as a charge stock for the process, a hydrocarbon oil boiling predominantly within or above the gasoline boiling range, for instance, boiling predominantly within in the range of from about 100° F. to about 750° F., and preferably predominantly within the range of from about 150° F. to about 450° F. However, processes using my catalyst can be advantageously applied to the dehydrogenation of lighter hydrocarbons such as ethane, propane, butane, isobutane, etc., to produce olefins for use in polymerization or other processes.

What I claim is:

1. A process for reforming naphtha to improve the antiknock quality thereof, which comprises contacting said naphtha, under reforming conditions of temperature and pressure, with a catalyst consisting of aluminum oxide and an alkali metal borate.

2. A process for the conversion of hydrocarbons into gasoline having improved antiknock qualities, which comprises heating said hydrocarbons to a temperature within the range of from about 950° F. to about 1050° F. under superatmospheric pressure, in the presence of a catalyst consisting of aluminum oxide and an alkali metal borate, and separating from the conversion products a fraction boiling within the gasoline boiling range.

3. A process for the conversion of hydrocarbons into gasoline having improved antiknock qual-

ties, which comprises heating said hydrocarbons to a temperature within the range of from about 950° F. to about 1050° F. under superatmospheric pressure, in the presence of a catalyst consisting of aluminum oxide and sodium borate, and separating from the conversion products a fraction boiling within the gasoline boiling range.

4. A process for the conversion of a hydrocarbon stock into other hydrocarbons, which comprises contacting said stock with a catalyst consisting of aluminum oxide and an alkali metal borate at a sufficiently elevated temperature to effect said conversion, said borate comprising from about 0.1% to about 10% by weight of said catalyst.

5. A process for the conversion of high boiling hydrocarbon oil into lower boiling hydrocarbons, which comprises subjecting said high boiling oil to cracking temperatures in the presence of a catalyst consisting of aluminum oxide and an alkali metal borate.

6. A process for the conversion of hydrocarbons into gasoline having improved antiknock qualities, which comprises heating said hydrocarbons to a temperature within the range of from about 950° F. to about 1050° F., in the presence of a catalyst consisting of aluminum oxide and sodium borate, and separating from the conversion products a fraction boiling within the gasoline boiling range.

7. A process for the conversion of a hydrocarbon stock into other hydrocarbons, which comprises contacting said stock with a catalyst consisting of aluminum oxide and an alkali metal borate at a temperature between 850° F. and 1050° F., and at a space velocity of from 1 to 4 volumes of stock per volume of catalyst per hour, said borate comprising from 0.1% to about 10% by weight of said catalyst.

ERNEST M. MARKS.